



US00754736B2

(12) **United States Patent**  
**Lin et al.**

(10) **Patent No.:** **US 7,547,366 B2**  
(45) **Date of Patent:** **\*Jun. 16, 2009**

(54) **2000 SERIES ALLOYS WITH ENHANCED DAMAGE TOLERANCE PERFORMANCE FOR AEROSPACE APPLICATIONS**

(75) Inventors: **Jen C. Lin**, Export, PA (US); **John M. Newman**, Export, PA (US); **Paul E. Magnusen**, Pittsburgh, PA (US); **Gary H. Bray**, Murrysville, PA (US)

(73) Assignee: **Alcoa Inc.**, Pittsburgh, PA (US)

(\*) Notice: Subject to any disclaimer, the term of this patent is extended or adjusted under 35 U.S.C. 154(b) by 0 days.

This patent is subject to a terminal disclaimer.

(21) Appl. No.: **10/893,003**

(22) Filed: **Jul. 15, 2004**

(65) **Prior Publication Data**

US 2006/0011272 A1 Jan. 19, 2006

(51) **Int. Cl.**  
**C22C 21/12** (2006.01)

(52) **U.S. Cl.** ..... **148/417**; 420/533; 420/539

(58) **Field of Classification Search** ..... 148/417;  
420/532, 533, 539, 534, 535

See application file for complete search history.

(56) **References Cited**

U.S. PATENT DOCUMENTS

3,925,067 A 12/1975 Sperry et al.  
5,211,910 A \* 5/1993 Pickens et al. ..... 420/532  
5,213,639 A 5/1993 Colvin et al.  
5,376,192 A 12/1994 Cassada, III  
5,512,112 A 4/1996 Cassada, III

5,593,516 A 1/1997 Cassada, III  
5,630,889 A 5/1997 Karabin et al.  
5,652,063 A 7/1997 Karabin  
5,665,306 A 9/1997 Karabin  
5,800,927 A 9/1998 Karabin  
5,863,359 A 1/1999 Karabin et al.  
5,865,914 A 2/1999 Karabin et al.

(Continued)

FOREIGN PATENT DOCUMENTS

GB 1320271 6/1973

(Continued)

OTHER PUBLICATIONS

"Aluminum and Aluminum Alloys", ASM International, 1993, p. 41.\*

(Continued)

*Primary Examiner*—Roy King

*Assistant Examiner*—Janelle Morillo

(74) *Attorney, Agent, or Firm*—Greenberg Traurig LLP

(57) **ABSTRACT**

The invention provides a 2000 series aluminum alloy having enhanced damage tolerance, the alloy consisting essentially of about 3.0-4.0 wt % copper; about 0.4-1.1 wt % magnesium; up to about 0.8 wt % silver; up to about 1.0 wt % Zn; up to about 0.25 wt % Zr; up to about 0.9 wt % Mn; up to about 0.5 wt % Fe; and up to about 0.5 wt % Si, the balance substantially aluminum, incidental impurities and elements, said copper and magnesium present in a ratio of about 3.6-5 parts copper to about 1 part magnesium. The alloy is suitable for use in wrought or cast products including those used in aerospace applications, particularly sheet or plate structural members, extrusions and forgings, and provides an improved combination of strength and damage tolerance.

**23 Claims, 5 Drawing Sheets**



# US 7,547,366 B2

Page 2

---

## U.S. PATENT DOCUMENTS

5,879,475 A 3/1999 Karabin  
6,368,427 B1 4/2002 Sigworth  
6,444,058 B1 9/2002 Liu et al.  
7,214,279 B2 \* 5/2007 Fischer et al. .... 148/417  
7,229,508 B2 \* 6/2007 Cho et al. .... 148/417  
7,229,509 B2 \* 6/2007 Cho .... 148/417  
2004/0071586 A1 \* 4/2004 Rioja et al. .... 420/532

## FOREIGN PATENT DOCUMENTS

JP 0317440 A \* 5/1991  
JP 03107440 5/1991

WO WO 2004003244 A1 \* 1/2004  
WO 2006019946 2/2006

## OTHER PUBLICATIONS

J. Schijve, "The significance of light-simulation fatigue tests," Delft University Report (LR-466), Jun. 1985.  
"After Concorde: Evaluation of an Al—Cu—Mg—Ag Alloy for Use in the Proposed European SST", Polmear I. J. et al, Materials Science Forum, Aedermannsdorf, CH, vol. 217-222, pp. 1759-1764, XPOO9003900, ISSN: 0255-5476.

International Search Report dated Oct. 1, 2007 relating to PCT/US06/034664.

\* cited by examiner



FIG. 1



FIG. 2

 $\Delta K$  (MPa $\sqrt{m}$ )







## 1

**2000 SERIES ALLOYS WITH ENHANCED  
DAMAGE TOLERANCE PERFORMANCE  
FOR AEROSPACE APPLICATIONS**

FIELD OF THE INVENTION

This invention relates to an Al—Cu—Mg—Ag-alloy having improved damage tolerance, suitable for aerospace and other demanding applications. The alloy has very low levels of iron and silicon, and a low copper to magnesium ratio.

BACKGROUND INFORMATION

In commercial jet aircraft applications, a key structural requirement for lower wing and fuselage applications is a high level of damage tolerance as measured by fatigue crack growth (FCG), and fracture toughness. Current generation materials are taken from the Al—Cu 2XXX family, typically of the 2X24 type. These alloys are usually used in a T3X temper and inherently have moderate strength with high fracture toughness and good FCG resistance. Typically, when the 2X24 alloys are artificially aged to a T8 temper, where strength is increased, there is a degradation in toughness and/or FCG performance.

Damage tolerance is a combination of fracture toughness and FCG resistance. As strength increases there is a concurrent decrease in fracture toughness, and maintaining high toughness with increased strength is a desirable attribute of any new alloy product. FCG performance is often measured using two common loading configurations: 1) constant amplitude (CA), and 2) under spectrum or variable loading. The latter is intended to better represent the loading expected in service. Details on flight simulated loading FCG tests are described in J. Schijve, "The significance of flight-simulation fatigue tests", Delft University Report (LR-466), June 1985. Constant amplitude FCG tests are run using a stress range defined by the R ratio, i.e. minimum/maximum stress. Crack growth rates are measured as a function of a stress intensity range (? K). Under spectrum loading, crack growth is again measured, but this time is reported over a number of "flights." Loading is such that it simulates typical takeoff, in flight, and landing loads for each flight, and this is repeated to represent typical lifetime loadings seen for a given part of the aircraft structure. The spectrum FCG tests are a more representative measure of an alloy's performance as they simulate actual aircraft operation. There are a number of generic spectrum loading configurations and also aircraft-specific spectrum which are dependent on aircraft design philosophy and also aircraft size. Smaller, single aisle aircraft are expected to have a higher number of takeoff/landing cycles than large, wide-bodied aircraft that make fewer but longer flights.

Under spectrum loading, an increase in yield strength will often reduce the amount of plasticity-induced crack closure (which retards crack propagation) and will typically result in lower lives. An example has been the performance of a recently developed High Damage Tolerant alloy (designated herein as 2X24HDT) which exhibits a superior spectrum life performance in the lower yield strength T351 temper versus the higher strength T39 temper. Aircraft designers would ideally like to have alloys that possess higher static properties (tensile strength) with the same or higher level of damage tolerance as that seen in the 2X24-T3 temper products.

U.S. Pat. No. 5,652,063 discloses an aluminum alloy composition having Al—Cu—Mg—Ag, in which the Cu—Mg ratio is in the range of about 5-9, with silicon and iron levels up to about 0.1 wt % each. The composition of the '063 patent

## 2

provides adequate strength, but unexceptional fracture toughness and resistance to fatigue crack growth.

U.S. Pat. No. 5,376,192 also discloses an Al—Cu—Mg—Ag aluminum alloy, having a Cu—Mg ratio of between about 2.3-25, and much higher levels of Fe and Si, on the order of up to about 0.3 and 0.25, respectively.

There remains a need for alloy compositions having adequate strength in combination with enhanced damage tolerance, including fracture toughness and improved resistance to fatigue crack growth, especially under spectrum loading.

SUMMARY OF THE INVENTION

The present invention solves the above need by providing a new alloy showing excellent strength with equal or better toughness and improved FCG resistance, particularly under spectrum loading, as compared with prior art compositions and registered alloys such as 2524-T3 for sheet (fuselage) and 2024-T351/2X24HDT-T351/2324-T39 for plate (lower wing). As used herein, the term "enhanced damage tolerance" refers to these improved properties.

Accordingly, the present invention provides an aluminum-based alloy having enhanced damage tolerance consisting essentially of about 3.0-4.0 wt % copper; about 0.4-1.1 wt % magnesium; up to about 0.8 wt % silver; up to about 1.0 wt % Zn; up to about 0.25 wt % Zr; up to about 0.9 wt % Mn; up to about 0.5 wt % Fe; and up to about 0.5 wt % Si; the balance substantially aluminum, incidental impurities and elements, said copper and magnesium present in a ratio of about 3.6-5 parts copper to about 1 part magnesium. Preferably, the aluminum-based alloy is substantially vanadium free. The Cu:Mg ratio is maintained at about 3.6-5 parts copper to 1 part magnesium, more preferably 4.0-4.5 parts copper to 1 part magnesium. While not wishing to be bound by any theory, it is thought that this ratio imparts the desired properties in the products made from the alloy composition of the present invention.

In an additional aspect, the invention provides a wrought or cast product made from an aluminum-based alloy consisting essentially of about 3.0-4.0 wt % copper; about 0.4-1.1 wt % magnesium; up to about 0.8 wt % silver; up to about 1.0 wt % Zn; up to about 0.25 wt % Zr; up to about 0.9 wt % Mn; up to about 0.5 wt % Fe; and up to about 0.5 wt % Si; the balance substantially aluminum, incidental impurities and elements, said copper and magnesium present in a ratio of about 3.6-5 parts copper to about 1 part magnesium. Preferably, the copper and magnesium are present in a ratio of about 4-4.5 parts copper to about 1 part magnesium. Also preferably, the wrought or cast product made from the aluminum-based alloy is substantially vanadium free.

It is an object of the present invention, therefore, to provide an aluminum alloy composition having improved combinations of strength, fracture toughness and resistance to fatigue.

It is an additional object of the present invention to provide wrought or cast aluminum alloy products having improved combinations of strength, fracture toughness and resistance to fatigue.

It is an object of the present invention to provide an aluminum alloy composition having improved combinations of strength, fracture toughness and resistance to fatigue, the alloy having a low Cu:Mg ratio.

These and other objects of the present invention will become more readily apparent from the following figures, detailed description and appended claims.

#### BRIEF DESCRIPTION OF THE DRAWINGS

The invention is further illustrated by the following drawings in which:

FIG. 1 is a graph showing constant amplitude FCG data for 2524-T3 and Sample A-T8 sheet. Tests were conducted in the T-L orientation with R ratio equals 0.1.

FIG. 2 is a graph showing constant amplitude FCG data for 2524-T3 and Sample A-T8 sheet. Tests were conducted in the L-T orientation with R ratio equals 0.1.

FIG. 3 is a graph showing constant amplitude FCG data for 2X24HDT-T39, 2X24HDT-T89, and Sample A plate. Tests were conducted in the L-T orientation with R ratio equal 0.1.

FIG. 4 is a graph showing comparison data of spectrum lives as a function of yield stress (by alloy/temper) for Sample A and Sample B plate and 2X24HDT.

FIG. 5 is a graph showing a comparison of fracture toughness as a function of yield stress (by alloy/temper) for Sample A and Sample B plate and 2X24HDT.

#### DETAILED DESCRIPTION OF PREFERRED EMBODIMENTS

Definitions: For the description of alloy compositions that follow, all references to percentages are by weight percent (wt %) unless otherwise indicated. When referring to a minimum (for instance for strength or toughness) or to a maximum (for instance for fatigue crack growth rate), these refer to a level at which specifications for materials can be written or a level at which a material can be guaranteed or a level that an airframe builder (subject to a safety factor) can rely on in design. In some cases, it can have a statistical basis, e.g., 99% of the product conforms or is expected to conform with 95% confidence using standard statistical methods.

When referring to any numerical range of values herein, such ranges are understood to include each and every number and/or fraction between the stated range minimum and maximum. A range of about 3.0-4.0 wt % copper, for example, would expressly include all intermediate values of about 3.1, 3.12, 3.2, 3.24, 3.5, all the way up to and including 3.61, 3.62, 3.63 and 4.0 wt % Cu. The same applies to all other elemental ranges set forth below, such as the Cu:Mg ratio of between about 3.6 and 5.

The present invention provides an aluminum-based alloy having enhanced damage tolerance consisting essentially of about 3.0-4.0 wt % copper; about 0.4-1.1 wt % magnesium; up to about 0.8 wt % silver; up to about 1.0 wt % Zn; up to about 0.25 wt % Zr; up to about 0.9 wt % Mn; up to about 0.5 wt % Fe; and up to about 0.5 wt % Si; the balance substantially aluminum, incidental impurities and elements, said copper and magnesium present in a ratio of about 3.6-5 parts copper to about 1 part magnesium. Preferably, the copper and magnesium are present in a ratio of about 4-4.5 parts copper to about 1 part magnesium.

As used herein, the term "substantially-free" means having no significant amount of that component purposefully added to the composition to import a certain characteristic to that alloy, it being understood that trace amounts of incidental elements and/or impurities may sometimes find their way into a desired end product. For example, a substantially vanadium-free alloy should contain less than about 0.1% V, or more preferably less than about 0.05% V due to contamination from incidental additives or through contact with certain

processing and/or holding equipment. All preferred first embodiments of this invention are substantially vanadium-free.

The aluminum-based alloy of the present invention optionally further comprises a grain refiner. The grain refiner can be titanium or a titanium compound, and when present, is present in an amount ranging up to about 0.1 wt %, more preferably about 0.01-0.05 wt %. All weight percentages for titanium, as used herein, refer to the amount of titanium or the amount containing titanium, in the case of titanium compounds, as would be understood by one skilled in the art. Titanium is used during the DC casting operation to modify and control the as-cast grain size and shape, and can be added directly into the furnace or as grain refiner rod. In the case of grain refiner rod additions, titanium compounds can be used, including, but not limited to,  $TiB_2$  or  $TiC$ , or other titanium compounds known in the art. The amount added should be limited, as excess titanium additions can lead to insoluble second phase particles which are to be avoided.

More preferred amounts of the various compositional elements of the above alloy composition include the following: magnesium present in an amount ranging from about 0.6-1.1 wt %; silver present in an amount ranging from about 0.2-0.7 wt %; and zinc present in an amount ranging up to about 0.6 wt %. Alternatively, zinc can be partially substituted for silver, with a combined amount of zinc and silver up to about 0.9 wt %.

Dispersoid additions can be made to the alloy to control the evolution of grain structure during hot working operations such as hot rolling, extrusion, or forging. One dispersoid addition can be zirconium, which forms  $Al_3Zr$  particles that inhibit recrystallization. Manganese can also be added, to replace zirconium or in addition to zirconium so as to provide a combination of two dispersoid forming elements that allow improved grain structure control in the final product. Manganese is known to increase the second phase content of the final product which can have a detrimental impact on fracture toughness; hence the level of additions made will be controlled to optimize alloy properties.

Preferably, zirconium will be present in an amount ranging up to about 0.18 wt %; manganese will more preferably be present in an amount ranging up to about 0.6 wt %, most preferably about 0.3-0.6 wt %. The final product form will influence the preferred range for the selected dispersoid additions.

Optionally, the aluminum-based alloy of the present invention further comprises scandium, which can be added as a dispersoid or grain refining element to control grain size and grain structure. When present, scandium will be added in an amount ranging up to about 0.25 wt %, more preferably up to about 0.18 wt %.

Other elements that can be added during casting operations include, but are not limited to, beryllium and calcium. These elements are used to control or limit oxidation of the molten aluminum. These elements are regarded as trace elements with additions typically less than about 0.01 wt %, with preferred additions less than about 100 ppm.

The alloys of the present invention have preferred ranges of other elements that are typically viewed as impurities and are maintained within specified ranges. Most common of these impurity elements are iron and silicon, and where high levels of damage tolerance are required (as in aerospace products) the Fe and Si levels are preferably kept relatively low to limit the formation of the constituent phases  $Al_1Cu_2Fe$  and  $Mg_2Si$  which are detrimental to fracture toughness and fatigue crack growth resistance. These phases have low solid solubility in Al-alloy and once formed cannot be eliminated by thermal

treatments. Additions of Fe and Si are maintained at less than about 0.5 wt % each. Preferably these are kept below a combined maximum level of less than about 0.25 wt %, with a more preferred combined maximum of less than about 0.2 wt % for aerospace products. Other incidental elements/impurities could include sodium, chromium or nickel, for example.

In an additional aspect, the invention provides a wrought or cast product made from an aluminum-based alloy consisting essentially of about 3.0-4.0 wt % copper; about 0.4-1.1 wt % magnesium; up to about 0.8 wt % silver; up to about 1.0 wt % Zn; up to about 0.25 wt % Zr; up to about 0.9 wt % Mn; up to about 0.5 wt % Fe; and up to about 0.5 wt % Si; the balance substantially aluminum, incidental impurities and elements, said copper and magnesium present in a ratio of about 3.6-5 parts copper to about 1 part magnesium. Preferably, the copper and magnesium are present in a ratio of about 4-4.5 parts copper to about 1 part magnesium. Also preferably, the wrought or cast product made from the aluminum-based alloy is substantially vanadium free. Additional preferred embodiments are those as described above for the alloy composition.

As used herein, the term "wrought product" refers to any wrought product as that term is understood in the art, including, but not limited to, rolled products such as forgings, extrusions, including rod and bar, and the like. A preferred category of wrought product is an aerospace wrought product, such as sheet or plate used in aircraft fuselage or wing manufacturing, or other wrought forms suitable for use in aerospace applications, as that term would be understood by one skilled in the art. Alternatively an alloy of the present invention may be used in any of the above-mentioned wrought forms in other products, such as products for other industries including automotive and other transportation applications, recreation/sports, and other uses. In addition, the inventive alloy may also be used as a casting alloy, as that term is understood in the art, where a shape is produced.

In an additional aspect, the present invention provides a matrix or metal matrix composite product, made from the alloy composition described above.

In accordance with the invention, a preferred alloy is made into an ingot-derived product suitable for hot working or rolling. For instance, large ingots of the aforesaid composition can be semicontinuously cast, then scalped or machined to remove surface imperfections as needed or required to provide a good rolling surface. The ingot may then be pre-heated to homogenize and solutionize its interior structure. A suitable preheat treatment is to heat the ingot to about 900-980° F. It is preferred that homogenization be conducted at cumulative hold times on the order of about 12 to 24 hours.

The ingot is then hot rolled to achieve a desired product dimensions. Hot rolling should be initiated when the ingot is at a temperature substantially above about 850° F., for instance around 900-950° F. For some products, it is preferred to conduct such rolling without reheating i.e. using the power of the rolling mill to maintain rolling temperatures above a desired minimum. Hot rolling is then continued, normally in a reversing hot mill, until the desired thickness of end plate product is achieved.

In accordance with this invention, the desired thickness of hot rolled plate for lower wing skin applications is generally between about 0.35 to 2.2 inches or so, and preferably within about 0.9 to 2 inches. Aluminum Association guidelines define sheet products as less than 0.25 inches in thickness; products above 0.25 inches are defined as plate.

In addition to the preferred embodiments of this invention for lower wing skin and spar webs, other applications of this alloy may include stringer extrusions. When making an extrusion, an alloy of the present invention is first heated to

between about 650-800° F., preferably about 675-775° F. and includes a reduction in cross-sectional area (or extrusion ratio) of at least about 10:1.

Hot rolled plate or other wrought product forms of this invention are preferably solution heat treated (SHT) at one or more temperatures between about 900° F. to 980° F. with the objective to take substantial portions, preferably all or substantially all, of the soluble magnesium and copper into solution, it being again understood that with physical processes which are not always perfect, probably every last vestige of these main alloying ingredients may not be fully dissolved during the SHT (or solutionizing) step(s). After heating to the elevated temperatures described above, the plate product of this invention should be rapidly cooled or quenched to complete solution heat treating. Such cooling is typically accomplished by immersion in a suitably sized tank of water or by using water sprays, although air chilling may be used as supplementary or substitute cooling means.

After quenching, this product can be either cold worked and/or stretched to develop adequate strength, relieve internal stresses and straighten the product. Cold deformation (for example cold rolling, cold compression) levels can be up to around 11% with a preferred range of about 8 to 10%. The subsequent stretching of this cold worked product will be up to a maximum of about 2%. In the absence of cold rolling the product may be stretched up to a maximum of about 8% with a preferred level of stretch in the 1 to 3% range.

After rapid quenching, and cold working if desired, the product is artificially aged by heating to an appropriate temperature to improve strength and other properties. In one preferred thermal aging treatment, the precipitation hardenable plate alloy product is subjected to one aging step, phase or treatment. It is generally known that ramping up to and/or down from a given or target treatment temperature, in itself, can produce precipitation (aging) effects which can, and often need to be, taken into account by integrating such ramping conditions and their precipitation hardening effects into the total aging treatment. Such integration is described in greater detail in U.S. Pat. No. 3,645,804 to Ponchel. With ramping and its corresponding integration, two or three phases for thermally treating the product according to the aging practice may be effected in a single, programmable furnace for convenience purposes, however, each stage (step or phase) will be more fully described as a distinct operation. Artificial aging treatments can use a single principal aging stage such up to 375° F. with aging treatments in a preferred range of 290 to 330° F. Aging times can range up to 48 hours with a preferred range of about 16 to 36 hours as determined by the artificial aging temperature.

A temper designation system has been developed by the Aluminum Association and is in common usage to describe the basic sequence of steps used to produce different tempers. In this system the T3 temper is described as solution heat treated, cold worked and naturally aged to a substantially stable condition, where cold work used is recognized to affect mechanical property limits. The T6 designation includes products that are solution heat treated and artificially aged, with little or no cold work such that the cold work is not thought to affect mechanical property limits. The T8 temper designates products that are solution heat treated, cold worked and artificially aged, where the cold work is understood to affect mechanical property limits.

Preferably, the product is a T6 or T8 type temper, including any of the T6 or T8 series. Other suitable tempers include, but are not limited to, T3, T39, T351, and other tempers in the T3X series. It is also possible that the product be supplied in a T3X temper and be subjected to a deformation or forming

process by an aircraft manufacturer to produce a structural component. After such an operation the product may be used in the T3X temper or aged to a T8X temper.

Age forming can provide a lower manufacturing cost while allowing more complex wing shapes to be formed. During age forming, the part is constrained in a die at an elevated temperature, usually between about 250° F. and about 400° F., for several to tens of hours, and desired contours are accomplished through stress relaxation. If a higher temperature artificial aging treatment is to be used, such as a treatment above 280° F., the metal can be formed or deformed into a desired shape during the artificial aging treatment. In general, most deformations contemplated are relatively simple, such as a very mild curvature across the width and/or length of a plate member.

In general, plate material is heated to about 300° F.-400° F., for instance around 310° F., and is placed upon a convex form and loaded by clamping or load application at opposite edges of the plate. The plate more or less assumes the contour of the form over a relatively brief period of time but upon cooling springs back a little when the force or load is removed. The curvature or contour of the form is slightly exaggerated with respect to the desired forming of the plate to compensate for springback. If desired, a low temperature artificial aging treatment step at around 250° F. can precede and/or follow age forming. Alternatively, age forming can be performed at a temperature such as about 250° F., before or after aging at a higher temperature such as about 330° F. One skilled in the art can determine the appropriate order and temperatures of each step, based on the properties desired and the nature of the end product.

The plate member can be machined after any step, for instance, such as by tapering the plate such that the portion intended to be closer to the fuselage is thicker and the portion closest to the wing tip is thinner. Additional machining or other shaping operations, if desired, can also be performed either before or after the age forming treatment.

Prior art lower wing cover material for the last few generations of modern commercial jetliners has been generally from the 2X24 alloy family in the naturally aged tempers such as T351 or T39, and thermal exposure during age forming is minimized to retain the desirable material characteristics of naturally aged tempers. In contrast, alloys of the present

invention are used preferably in the artificially aged tempers, such as T6 and T8-type tempers, and the artificial aging treatment can be simultaneously accomplished during age forming without causing any degradation to its desirable properties. The ability of the invention alloy to accomplish desired contours during age forming is either equal to or better than the currently used 2X24 alloys.

## EXAMPLE

10

In preparing inventive alloy compositions to illustrate the improvement in mechanical properties, ingots of 6×16 inch cross-section were Direct Chill (D.C.) cast for the Sample A to D compositions defined in Tables 1 and 2. After casting the ingots were scalped to about 5.5 inch thickness in preparation for homogenization and hot rolling. The ingots were batch homogenized using a multi-step practice with a final step of soaking at about 955 to 965° F. for 24 hrs. The ingots were given an initial hot rolling to an intermediate slab gage and then reheated at about 940° F. to completed the hot rolling operation, reheating was used when hot rolling temperatures fell below about 700° F. The samples were hot rolled to about 0.75 inches for the plate material and about 0.18 inches for sheet. After hot rolling the sheet samples were cold rolled about 30% to finish at about 0.125 inches in gage.

Samples of the fabricated plate and sheet were then heat treated, at temperatures in the range of about 955 to 965° F. using soak times of up to 60 minutes, and then cold water quenched. The plate samples were stretched within one hour of the quench to a nominal level of about 2.2%. The sheet samples were also stretched within one hour of the quench with a nominal level of about 1% used. Samples of the plate and sheet were allowed to naturally age after stretching for about 72 hours before being artificially aged. Samples were artificially aged for between 24 and 32 hours at about 310° F. The sample plates and sheets were then characterized for mechanical properties including tensile, fracture toughness and fatigue crack growth resistance.

Tables 1 and 2 show sheet and plate products made from compositions of the present invention as compared with prior art compositions.

TABLE 1

| Al—Cu—Mg—Ag (Plate)<br>Alloy   | Composition |            |            |            |            |           |            |            |            |
|--------------------------------|-------------|------------|------------|------------|------------|-----------|------------|------------|------------|
|                                | Cu<br>wt %  | Mg<br>wt % | Ag<br>Wt % | Zn<br>wt % | Mn<br>wt % | V<br>wt % | Zr<br>wt % | Si<br>wt % | Fe<br>wt % |
| Sample F<br>(per Karabin)      | 5           | 0.8        | 0.55       | 0          | 0.6        | 0         | 0.13       | 0.06       | 0.07       |
| Sample E<br>(per Cassada)      | 4.5         | 0.7        | 0.5        | <0.05      | 0.3        | <0.05     | 0.11       | 0.04       | 0.06       |
| Sample D                       | 4.9         | 0.8        | 0.48       | <0.05      | 0.3        | <0.05     | 0.11       | 0.02       | 0.01       |
| Sample C                       | 4.7         | 1.0        | 0.51       | <0.05      | 0.3        | <0.05     | 0.11       | 0.06       | 0.03       |
| Sample B                       | 3.6         | 0.8        | 0.48       | <0.05      | 0.3        | <0.05     | 0.09       | 0.03       | 0.02       |
| Sample A                       | 3.6         | 0.9        | 0.48       | <0.05      | 0.3        | <0.05     | 0.12       | 0.02       | 0.03       |
| 2×24 HDT<br>(Commercial Alloy) | 3.8-4.3     | 1.2-1.63   | <0.05      | <0.05      | 0.45-0.7   | <0.05     | <0.05      |            |            |
| 2324<br>(Commercial Alloy)     | 3.8-4.4     | 1.2-1.8    | <0.05      | <0.05      | 0.30-0.9   | <0.05     | <0.05      |            |            |

TABLE 2

| Al—Cu—Mg—Ag (Sheet) Alloy | Composition |         |         |         |          |        |         |         |         |
|---------------------------|-------------|---------|---------|---------|----------|--------|---------|---------|---------|
|                           | Cu wt %     | Mg wt % | Ag wt % | Zn wt % | Mn wt %  | V wt % | Zr wt % | Fe wt % | Si wt % |
| Sample F (per Karabin)    | 5           | 0.8     | 0.55    | 0       | 0.6      | 0      | 0.13    | 0.07    | 0.06    |
| Sample E (per Cassada)    | 4.5         | 0.7     | .5      | <0.05   | 0.3      | <0.05  | <0.11   | 0.06    | 0.04    |
| Sample D                  | 4.9         | 0.8     | 0.48    | <0.05   | 0.3      | <0.05  | <0.11   | 0.01    | 0.02    |
| Sample C                  | 4.7         | 1.0     | 0.51    | <0.05   | 0.3      | <0.05  | <0.11   | 0.03    | 0.06    |
| Sample B                  | 3.6         | 0.8     | 0.48    | <0.05   | 0.3      | <0.05  | <0.09   | 0.02    | 0.03    |
| Sample A                  | 3.6         | 0.9     | 0.48    | <0.05   | 0.3      | <0.05  | <0.12   | 0.03    | 0.02    |
| 2524 (Commercial Alloy)   | 4.0-4.5     | 1.2-1.6 | <0.05   | <0.05   | 0.45-0.7 | <0.05  | <0.05   |         |         |

## Fatigue Crack Growth Resistance

An important property to airframe designers is resistance to cracking by fatigue. Fatigue cracking occurs as a result of repeated loading and unloading cycles, or cycling between a high and a low load such as when a wing moves up and down or a fuselage swells with pressurization and contracts with depressurization. The loads during fatigue are below the static ultimate or tensile strength of the material measured in a tensile test and they are typically below the yield strength of the material. If a crack or crack-like defect exists in a structure, repeated cyclic or fatigue loading can cause the crack to grow. This is referred to as fatigue crack propagation. Propagation of a crack by fatigue may lead to a crack large enough to propagate catastrophically when the combination of crack size and loads are sufficient to exceed the material's fracture toughness. Thus, an increase in the resistance of a material to crack propagation by fatigue offers substantial benefits to aerostructure longevity. The slower a crack propagates, the better. A rapidly propagating crack in an airplane structural member can lead to catastrophic failure without adequate time for detection, whereas a slowly propagating crack allows time for detection and corrective action or repair.

The rate at which a crack in a material propagates during cyclic loading is influenced by the length of the crack. Another important factor is the difference between the maximum and the minimum loads between which the structure is cycled. One measurement which takes into account both the crack length and the difference between maximum and minimum loads is called the cyclic stress intensity factor range or  $\Delta K$ , having units of ksi/in, similar to the stress intensity factor used to measure fracture toughness. The stress intensity factor range ( $\Delta K$ ) is the difference between the stress intensity factors at the maximum and minimum loads. Another measure of fatigue crack propagation is the ratio between the minimum and maximum loads during cycling, called the stress ratio and denoted by  $R$ , where a ratio of 0.1 means that the maximum load is 10 times the minimum load.

The crack growth rate can be calculated for a given increment of crack extension by dividing the change in crack length (called  $\Delta a$ ) by the number of loading cycles ( $\Delta N$ ) which resulted in that amount of crack growth. The crack propagation rate is represented by  $\Delta a/\Delta N$  or 'da/dN' and has units of inches/cycle. The fatigue crack propagation rates of a material can be determined from a center cracked tension panel.

Under spectrum loading conditions the results are sometimes reported as the number of simulated flights to cause

final failure of the test specimen but is more often reported as the number of flights necessary to grow the crack over a given increment of crack extension, the latter sometimes representing a structurally-significant length such as the initial inspectable crack length.

Specimen dimensions for the Constant Amplitude FCG performance testing of sheet were 4.0 inches wide by 12 inches in length by full sheet thickness. Spectrum tests were performed using a specimen of the same dimensions using a typical fuselage spectrum and the number of flights and the results presented in Table 3. As can be seen in Table 3, over a crack length interval from 8 to 35 mm the spectrum life can be increased by over 50% with the new alloy. The spectrum FCG tests were performed in the L-T orientation.

TABLE 3

| Alloy                       | Typical Spectrum FCG data for sheet material tested in the L-T orientation |                                |
|-----------------------------|----------------------------------------------------------------------------|--------------------------------|
|                             | Flights at<br>a = 8.0 mm                                                   | Flights from<br>a = 8 to 35 mm |
| A2524-T3                    | 14,068                                                                     | 37,824                         |
| Sample E-T8 (per Cassada)   | 11,564                                                                     | 29,378                         |
| Sample A-T8                 | 24,200                                                                     | 56,911                         |
| % improvement               |                                                                            |                                |
| Sample A-T8<br>over 2524-T3 | 72%                                                                        | 50%                            |

The new alloy was also tested under constant amplitude FCG conditions for both L-T and T-L orientations at  $R=0.1$  (FIGS. 1 and 2). The T-L orientation is usually the most critical for a fuselage application but in some areas such as the fuselage crown (top) over the wings, the L-T orientation becomes the most critical.

Improved performance is measured by having lower crack growth rates at a given  $\Delta K$  value. For all values tested the new alloy shows an enhanced performance over 2524-T3. FCG data is typically plotted on log-log scales which tends to minimize the degree of difference between the alloys. However, for a given  $\Delta K$  value, the improvement of alloy Sample A can be quantified as shown in Table 4 (FIG. 1):

TABLE 4

| Constant Amplitude FCG data for sheet material tested in the T-L orientation |             |                     |                                         |
|------------------------------------------------------------------------------|-------------|---------------------|-----------------------------------------|
| Alloy                                                                        | ? K (MPa/m) | FCG Rate (mm/cycle) | % Decrease in FCG Rate (Sample vs.2524) |
| 2524-T3                                                                      | 10          | 1.1 E-04            | —                                       |
| Sample A-T8                                                                  | 10          | 3.8 E-05            | 65%                                     |
| 2524-T3                                                                      | 20          | 6.5 E-04            | —                                       |
| Sample A-T8                                                                  | 20          | 4.6 E-04            | 29%                                     |
| 2524-T3                                                                      | 30          | 2.5 E-03            | —                                       |
| Sample A-T8                                                                  | 30          | 1.1 E-03            | 56%                                     |

Note:  
lower values of FCG rate are an indication of improved performance

The invention alloy was also tested in the plate form under both Constant Amplitude (CA), for Sample A, and spectrum loading (Samples A and B). Specimen dimensions for the CA tests were the same as those for sheet, except that the specimens were machined to a thickness of 0.25 inch from the mid-thickness (T/2) location by equal metal removal from both plate surfaces. For the spectrum tests, the specimen dimensions were 7.9 inches wide by 0.47 inches thick also from the mid-thickness (T/2) location. All tests were performed in the L-T orientation since this orientation corresponds to the principal direction of tension loading during flight.

As can be seen in FIG. 3, under CA loading the inventive alloy has faster FCG rates, particularly in the lower ? K regime, than the high damage tolerant alloy composition 2X24HDT in the T39 temper. When the 2X24HDT alloy is artificially aged to the T89 temper it exhibits a degradation in CA fatigue crack growth performance which is typical of 2X24 alloys. This is a principal reason the T39 and lower strength T351 tempers are almost exclusively used in lower wing application even though artificially aged tempers such as the T89, T851 or T87 offer many advantages such as ability to age form to the final temper and better corrosion resistance. The inventive alloy, even though in an artificially aged condition, has superior FCG resistance than 2X24HDT-T89 at all ? K, while exceeding the performance of 2X24HDT in the high damage tolerant T39 temper at higher ? K. The lower ? K regime in fatigue crack growth is significant as this is where the majority of structural life is expected to occur. Based on the superior CA performance of 2X24HDT in the T39 temper and similar yield strength it would be expected that it would be superior to Sample A under spectrum loading. Surprisingly, however, when tested under a typical lower wing spectrum, Sample A performed significantly better 2X24HDT-T39, exhibiting a 36% longer life (FIG. 4, Table 5). This result could not have been predicted by one skilled in the art. More surprisingly, the spectrum performance of Sample A was superior to that of 2X24HDT in the T351 temper which has similar constant amplitude FCG resistance to 2X24HDT-T39 but significantly lower yield strength than either 2X24HDT-T39 or Sample A. The superior spectrum performance of the inventive alloy is also shown by the data on Sample B (Table 5 and FIG. 4).

Those skilled in the art recognizing that lower yield strength is beneficial to spectrum performance as further illustrated by the trend line in FIG. 4 for 2X24HDT processed

to T3X tempers having a range of strength levels. The spectrum life of Samples A and B lie clearly above this trend line for 2X24HDT and also are clearly superior to the compositions of Cassada which lie below the trend line for 2X24HDT.

5

TABLE 5

| Typical Spectrum FCG data for plate material tested in the L-T orientation |                           |             |                                |                                                |
|----------------------------------------------------------------------------|---------------------------|-------------|--------------------------------|------------------------------------------------|
|                                                                            | Alloy                     | L TYS (ksi) | # of Flights (a = 25 to 65 mm) | Life Improvement of Sample A over 2x24-T39 (%) |
| 10                                                                         | 2X24HDT-T39               | 66          | 4952                           | —                                              |
| 15                                                                         | 2 x 24HDT-T351            | 54          | 5967                           | 20%                                            |
| 15                                                                         | Sample E (per Cassada)    | 58          | 5007                           | 1%                                             |
| 20                                                                         | Sample E (per Cassada)    | 71          | 4174                           | -16%                                           |
| 20                                                                         | Sample D-T8 (per Karabin) | 75          | 4859                           | -2%                                            |
| 20                                                                         | Sample C-T8               | 76          | 4877                           | -2%                                            |
| 20                                                                         | Sample B-T8               | 62          | 6287                           | 27%                                            |
| 20                                                                         | Sample A-T8               | 64          | 6745                           | 36%                                            |

### Fracture Toughness

The fracture toughness of an alloy is a measure of its resistance to rapid fracture with a preexisting crack or crack-like flaw present. Fracture toughness is an important property to airframe designers, particularly if good toughness can be combined with good strength. By way of comparison, the tensile strength, or ability to sustain load without fracturing, of a structural component under a tensile load can be defined as the load divided by the area of the smallest section of the component perpendicular to the tensile load (net section stress). For a simple, straight-sided structure, the strength of the section is readily related to the breaking or tensile strength of a smooth tensile coupon. This is how tension testing is done. However, for a structure containing a crack or crack-like defect, the strength of a structural component depends on the length of the crack, the geometry of the structural component, and a property of the material known as the fracture toughness. Fracture toughness can be thought of as the resistance of a material to the harmful or even catastrophic propagation of a crack under a tensile load.

Fracture toughness can be measured in several ways. One way is to load in tension a test coupon containing a crack. The load required to fracture the test coupon divided by its net section area (the cross-sectional area less the area containing the crack) is known as the residual strength with units of thousands of pounds force per unit area (ksi). When the strength of the material as well as the specimen are constant, the residual strength is a measure of the fracture toughness of the material. Because it is so dependent on strength and geometry, residual strength is usually used as a measure of fracture toughness when other methods are not as useful because of some constraint like size or shape of the available material.

When the geometry of a structural component is such that it doesn't deform plastically through the thickness when a tension load is applied (plane-strain deformation), fracture toughness is often measured as plane-strain fracture tough-

ness,  $K_{Ic}$ . This normally applies to relatively thick products or sections, for instance 0.6 or 0.75 or 1 inch or more. ASTM E-399 has established a standard test using a fatigue pre-cracked compact tension specimen to measure  $K_{Ic}$ , which has the units ksi/in. This test is usually used to measure fracture toughness when the material is thick because the test is believed to be independent of specimen geometry as long as appropriate standards for width, crack length and thickness are met. The symbol K, as used in  $K_{Ic}$ , is referred to as the stress intensity factor.

Structural components which deform by plane-strain are relatively thick as indicated above. Thinner structural components (less than 0.6 to 0.75 inch thick) usually deform under plane stress or more usually under a mixed mode condition. Measuring fracture toughness under this condition can introduce additional variables because the number which results from the test depends to some extent on the geometry of the test coupon. One test method is to apply a continuously increasing load to a rectangular test coupon containing a crack. A plot of stress intensity versus crack extension known as an R-curve (crack resistance curve) can be obtained this way. R-curve determination is set forth in ASTM E561.

When the geometry of the alloy product or structural component is such that it permits deformation plastically through its thickness when a tension load is applied, fracture toughness is often measured as plane-stress fracture toughness. The fracture toughness measure uses the maximum load generated on a relatively thin, wide pre-cracked specimen. When the crack length at the maximum load is used to calculate the stress-intensity factor at that load, the stress-intensity factor is referred to as plane-stress fracture toughness  $K_c$ . When the stress-intensity factor is calculated using the crack length before the load is applied, however, the result of the calculation is known as the apparent fracture toughness,  $K_{app}$ , of the material. Because the crack length in the calculation of  $K_c$  is usually longer, values for  $K_c$  are usually higher than  $K_{app}$  for a given material. Both of these measures of fracture toughness are expressed in the units ksi/in. For tough materials, the numerical values generated by such tests generally increase as the width of the specimen increases or its thickness decreases.

It is to be appreciated that the width of the test panel used in a toughness test can have a substantial influence on the stress intensity measured in the test. A given material may exhibit a  $K_{app}$  toughness of 60 ksi/in using a 6-inch wide test specimen, whereas for wider specimens the measured  $K_{app}$  will increase with the width of the specimen. For instance, the same material that had a 60 ksi/in  $K_{app}$  toughness with a 6-inch panel could exhibit higher  $K_{app}$  values, for instance around 90 ksi/in in a 16-inch panel, around 150 ksi/in in a 48-inch wide panel and around 180 ksi/in in a 60-inch wide panel. To a lesser extent, the measured Kapp value is influenced by the initial crack length (i.e., specimen crack length) prior to testing. One skilled in the art will recognize that direct comparison of K values is not possible unless similar testing procedures are used, taking into account the size of the test panel, the length and location of the initial crack, and other variables that influence the measured value.

Fracture toughness data have been generated using a 16" M(T) specimen. All K values for toughness in the following tables were derived from testing with a 16-inch wide panel

and a nominal initial crack length of 4.0 inches. All testing was carried out in accordance with ASTM E561 and ASTM B646.

As can be seen in Table 6 and FIG. 5, the new alloy (Samples A and B) has a significantly higher toughness (measured by Kapp) when compared to comparable strength alloys in the T3 temper. Thus, an alloy of the present invention can sustain a larger crack than a comparative alloy such as 10 2324-T39 in both thick and thin sections without failing by rapid fracture.

Alloy 2X24HDT-T39 has a typical yield strength (TYS) of ~66 ksi and a  $K_{app}$  value of 105 ksi/in, while the new alloy has a slightly lower TYS of ~64 ksi (3.5% lower) but a toughness  $K_{app}$  value of 120 ksi/in (12.5% higher). It can also be seen that when aged to a T8 temper, the 2X24HDT product shows a strength increase TYS ~70 ksi with a  $K_{app}$  value of 103 ksi/in. In sheet form an alloy of the present invention also 20 exhibits higher strength with high fracture toughness when compared to standard 2x24-T3 standard sheet products.

A complete comparison of the properties of alloys of the present invention and prior art alloys is shown in Tables 6, 7, 8 and 9.

TABLE 6

| Typical Tensile and Fracture Toughness data for the Plate Material |        |                    |              |          |                       |                |
|--------------------------------------------------------------------|--------|--------------------|--------------|----------|-----------------------|----------------|
| Al—Cu—Mg—Ag<br>(Plate)                                             | Temper | Tensile Properties |              |          | Fracture<br>Toughness |                |
|                                                                    |        | TYS<br>(ksi)       | UTS<br>(ksi) | E<br>(%) | Kapp<br>(ksi/in)      | KC<br>(ksi/in) |
| Alloy Sample F<br>(per Karabin)                                    | T8     | 68.7               | 75.3         | 13.0     | 106.6                 | 148.4          |
| Sample E<br>(per Cassada)                                          | T8     | 70.9               | 76.3         | 13.5     | 114.0                 | 166.0          |
| Sample D<br>(per Karabin)                                          | T8     | 75.6               | 78.9         | 12.0     | 109.0                 |                |
| Sample C                                                           | T8     | 74.6               | 78.1         | 11.5     | 113.0                 |                |
| Sample B                                                           | T8     | 61.8               | 67.8         | 17.5     | 117.0                 |                |
| Sample A                                                           | T8     | 63.8               | 70.1         | 16.5     | 120.0                 |                |
| 2 x 24 HDT-T39<br>(Commercial Alloy)                               | T39    | 66.0               | 70.4         | 13.7     | 105.0                 | 150.0          |
| 2 x 24 HDT-T351<br>(Commercial Alloy)                              | T351   | 54.0               | 67.1         | 21.9     | 102.0                 | 157.0          |
| 2324-T39<br>(Commercial Alloy)                                     | T39    | 66.5               | 69.0         | 11.0     | 98.0                  |                |

TABLE 7

| Typical Tensile Property data for the Sheet Material |        |                    |                 |             |
|------------------------------------------------------|--------|--------------------|-----------------|-------------|
| Al—Cu—Mg—Ag (Sheet)<br>Alloy                         | Temper | Tensile Properties |                 |             |
|                                                      |        | TYs (ksi)<br>LT    | UTS (ksi)<br>LT | E (%)<br>LT |
| Sample F (per Karabin)                               | T8     |                    |                 |             |
| Sample E (per Cassada)                               | T8     | 60.4               | 69.0            | 12.7        |
| Sample D (per Karabin)                               | T8     | 67.3               | 73.2            | 10.3        |
| Sample C                                             | T8     | 67.9               | 74.4            | 11.0        |
| Sample B                                             | T8     | 52.7               | 62.4            | 15.3        |
| Sample A                                             | T8     | 54.1               | 63.3            | 13.0        |
| 2524-T3<br>(Commercial Alloy)                        | T3     | 45.0               | 64.0            | 21.0        |

TABLE 8

Typical Constant Amplitude and Spectrum FCG results for the Plate Material

| Al—Cu—Mg—Ag (Plate)<br>Alloy          | Fatigue                                         |                                                   |                                                   |                                               |
|---------------------------------------|-------------------------------------------------|---------------------------------------------------|---------------------------------------------------|-----------------------------------------------|
|                                       | FCG Rate (da/dN)                                |                                                   |                                                   |                                               |
|                                       | Delta K<br>(ksi/in) @<br>10-6 in/cycle<br>(L-T) | Delta K<br>(ksi/in) @ 10-<br>5 in/cycle (L-<br>T) | Delta K<br>(ksi/in) @ 10-<br>4 in/cycle (L-<br>T) | Spectrum<br>No of<br>Flights at<br>Smf = 100% |
| Sample F (per Karabin)                | 7.3                                             | 11.9                                              | 23.4                                              |                                               |
| Sample E (per Cassada)                | 7.0                                             | 12.8                                              | 27.0                                              |                                               |
| Sample D (per Karabin)                | 7.2                                             | 13.1                                              | 29.7                                              | 4859                                          |
| Sample C                              | 7.4                                             | 13.3                                              | 28.7                                              | 4877                                          |
| Sample B                              | 8.1                                             | 13.8                                              | 31.3                                              | 6287                                          |
| Sample A                              | 8.0                                             | 12.8                                              | 32.9                                              | 6745                                          |
| 2 x 24HDT -T39<br>(Commercial Alloy)  | 9.1                                             | 14.4                                              | 27.0                                              | 4952                                          |
| 2 x 24HDT -T351<br>(Commercial Alloy) |                                                 | 13.6                                              |                                                   | 5967                                          |
| 2324-T39 (Commercial Alloy)           | 8.1                                             | 13.1                                              | 25.4                                              | —                                             |

TABLE 9

Typical Constant Amplitude and Spectrum FCG results for the Sheet Material

| Al—Cu—Mg—Ag (Sheet)<br>Alloy  | Fatigue                                         |                                                 |                                                 |          |
|-------------------------------|-------------------------------------------------|-------------------------------------------------|-------------------------------------------------|----------|
|                               | FCG Rate (da/dN)*                               |                                                 |                                                 |          |
|                               | Delta K<br>(ksi/in) @<br>10-6 in/cycle<br>(T-L) | Delta K<br>(ksi/in) @<br>10-5 in/cycle<br>(T-L) | Delta K<br>(ksi/in) @<br>10-6 in/cycle<br>(T-L) | Spectrum |
| Sample D (per Karabin)        | 6.8                                             | 14.4                                            | 35.7                                            |          |
| Sample C                      | 7.6                                             | 14.4                                            | 33.4                                            |          |
| Sample B                      | 8.1                                             | 13.3                                            | 37.2                                            |          |
| Sample A                      | 8.2                                             | 14.9                                            | 36.0                                            | 24200.0  |
| 2524-T3<br>(Commercial Alloy) | 6.5                                             | 13.1                                            | 27.5                                            | 14068.0  |
|                               |                                                 |                                                 |                                                 | 56911.0  |
|                               |                                                 |                                                 |                                                 | 37824.0  |

An alloy of the present invention exhibits improvements relative to 2324-T39 in both fatigue initiation resistance and fatigue crack growth resistance at low  $\Delta K$ , which allows the threshold inspection interval to be increased. This improvement provides an advantage to aircraft manufacturers by increasing the time to a first inspection, thus reducing operating costs and aircraft downtime. An alloy of the present invention also exhibits improvements relative to 2324-T39 in fatigue crack growth resistance and fracture toughness, properties relevant to the repeat inspection cycle, which primarily depends on fatigue crack propagation resistance of an alloy at medium to high  $\Delta K$  and the critical crack length which is determined by its fracture toughness. These improvements will allow an increase in the number of flight cycles between inspections. Due to the benefits provided by the present invention, aircraft manufacturers can also increase operating stress and reduce aircraft weight while maintaining the same inspection interval. The reduced weight may result in greater fuel efficiency, greater cargo and passenger capacity and/or greater aircraft range.

#### Additional Testing

Additional samples were prepared as follows: samples were cast into bookmolds of approximately 1.25×2.75 inch cross-section. After casting the ingots were scalped to about

1.1 inch thickness in preparation for homogenization and hot rolling. The ingots were batch homogenized using a multi-step practice with a final step of soaking at about 955 to 965° F. for 24 hrs. The scalped ingots were then given a heat-to-roll practice at about 825° F. and hot rolled down to about 0.1 inches in thickness. Samples were heat-treated, at temperatures in the range of about 955 to 965° F. using soak times of up to 60 minutes, and then cold water quenched. The samples were stretched within one hour of the quench to a nominal level of about 2%, allowed to naturally age after stretching for about 96 hours before being artificially aged for between about 24 and 48 hours at about 310° F. The samples were then characterized for mechanical properties including tensile and the Kahn tear (toughness-indicator) test. Results are presented in Table 10.

As can be seen in Table 10, additions of zinc when made to the alloy either in addition to or as a partial substitution for silver can lead to higher toughness for equal strength. Table 10 illustrates the toughness of the alloy as measured by a sub-scale toughness indicator test (Kahn-tear test) under the guidelines of ASTM B871. The results of this test are expressed as Unit of Propagation Energy (UPE) in units of inch-lb/in<sup>2</sup>, with a higher number being an indication of higher toughness. Sample 3 in Table 10 shows higher toughness when zinc is present as a partial substitute for silver as

compared to equal strength for Sample 1 when silver alone is added. The addition of zinc with silver can lead to equal or lower toughness for the same strength (Samples 1 and 2 compared to Samples 4 and 5). Additions of zinc without any silver can result in toughness levels obtained when silver alone is added, however, these toughness indicator levels are obtained at much lower strength levels (Sample 1 compared with Samples 6 through 9). The optimum combination of strength and toughness can be achieved by a preferred combination of copper, magnesium, silver, and zinc.

TABLE 10

| Alloy    | Chemical Analyses (in wt %) and typical tensile, and toughness indicator properties |     |     |      | TYS<br>(ksi) | UTS<br>(ksi) | E1<br>(%) | UPE<br>(in-lb/in <sup>2</sup> ) |
|----------|-------------------------------------------------------------------------------------|-----|-----|------|--------------|--------------|-----------|---------------------------------|
|          | Cu                                                                                  | Mg  | Ag  | Zn   |              |              |           |                                 |
| Sample 1 | 4.5                                                                                 | 0.8 | 0.5 |      | 70           | 73           | 13        | 617                             |
| Sample 2 | 4.5                                                                                 | 0.8 | 0.5 | 0.2  | 69           | 73           | 12        | 548                             |
| Sample 3 | 4.5                                                                                 | 0.8 | 0.3 | 0.2  | 69           | 75           | 11        | 720                             |
| Sample 4 | 3.5                                                                                 | 0.8 | 0.5 |      | 60           | 66           | 15        | 1251                            |
| Sample 5 | 3.5                                                                                 | 0.8 | 0.5 | 0.2  | 60           | 65           | 14        | 1176                            |
| Sample 6 | 4.5                                                                                 | 0.8 |     | 0.35 | 55           | 65           | 16        | 786                             |
| Sample 7 | 4.5                                                                                 | 0.8 |     | 0.58 | 60           | 68           | 14        | 619                             |
| Sample 8 | 4.5                                                                                 | 0.8 |     | 0.92 | 58           | 67           | 14        | 574                             |
| Sample 9 | 4.5                                                                                 | 0.5 |     | 0.91 | 55           | 63           | 13        | 704                             |

In aircraft structure there are numerous mechanical fasteners installed that allows the assembly of the fabricated materials into components. The fastened joints are usually a source of fatigue initiation and the performance of material in representative coupons with fasteners is a quantitative measure of alloy performance. One such test is the High Load Transfer (HLT) test that is representative of chord-wise joints in wing-skin structure. In such tests alloys of the current invention were tested against the 2X24HDT product (Table 11). The invention alloy (Sample A) has an average fatigue life that is 100% improved over the baseline material.

TABLE 11

| Typical High Load Transfer (HLT) joint fatigue lives |                                              |             |
|------------------------------------------------------|----------------------------------------------|-------------|
| Alloy                                                | Average HLT fatigue life (6 tests per alloy) | Improvement |
| 2 x 24HDT                                            | 55,748 cycles                                |             |
| Sample A                                             | 116,894 cycles                               | 100%        |

Whereas particular embodiments of this invention have been described above for purposes of illustration, it will be evident to those skilled in the art that numerous variations of the details of the present invention may be made without departing from the invention as defined in the appended claims.

What is claimed is:

1. A 2000 series aluminum-based alloy having enhanced damage tolerance consisting essentially of:  
about 3.0 to about 4.0 wt % copper;  
about 0.4 to about 1.1 wt % magnesium;  
about 0.2 to about 0.8 wt % silver;  
up to about 0.6 wt % Zn, wherein the zinc is partially substituted for the silver and a combined amount of zinc and silver is up to about 0.9 wt %;  
up to about 0.25 wt % Zr;  
up to about 0.9 wt % Mn;  
a combined Si and Fe content of about 0.25 wt % or less;

the balance substantially aluminum, incidental impurities and elements, said copper and magnesium present in a ratio of about 3.6-4.5 parts copper to about 1 part magnesium.

5 2. The aluminum-based alloy of claim 1, further comprising a grain refiner.

3. The aluminum-based alloy of claim 2, wherein said grain refiner is titanium or a titanium compound, and said titanium or titanium compound is present in an amount ranging up to 10 about 0.1 wt %.

4. The aluminum-based alloy of claim 1, wherein said zirconium is present in an amount ranging up to about 0.18 wt %.

15 5. The aluminum-based alloy of claim 1, wherein said manganese is present in an amount ranging from about 0.3-0.6 wt %.

6. The aluminum-based alloy of claim 1, wherein the combined amount of said iron and said silicon is up to about 0.25 wt %.

20 7. The aluminum-based alloy of claim 1, further comprising scandium.

8. The aluminum-based alloy of claim 7, wherein said scandium is present in amount ranging up to about 0.25 wt %.

9. The aluminum-based alloy of claim 1, further comprising an oxidation-controlling element.

10. The aluminum-based alloy of claim 9, wherein said oxidation-controlling element is beryllium or calcium.

11. A wrought or cast product made from an aluminum-based alloy having enhanced damage tolerance consisting 30 essentially of:

about 3.0 to about 4.0 wt % copper;  
about 0.4 to about 1.1 wt % magnesium;  
from about 0.2 to about 0.8 wt % silver;  
up to about 0.6 wt % Zn, wherein the zinc is partially substituted for the silver and a combined amount of zinc and silver is up to about 0.9 wt %;  
up to about 0.25 wt % Zr;  
up to about 0.9 wt % Mn;  
a combined Fe and Si content of up to about 0.25 wt % or less;

35 the balance substantially aluminum, incidental impurities and elements, said copper and magnesium present in a ratio of about 3.6-4.5 parts copper to about 1 part magnesium.

12. The wrought or cast product of claim 11, further comprising a grain refiner.

13. The wrought or cast product of claim 12, wherein said grain refiner is titanium or a titanium compound, and said titanium or titanium compound is present in an amount ranging up to about 0.1 wt %.

50 14. The wrought or cast product of claim 11, wherein said zirconium is present in an amount ranging up to about 0.18 wt %.

15. The wrought or cast product of claim 11, wherein said manganese is present in an amount ranging from about 0.3-0.6 wt %.

16. The wrought or cast product of claim 11, wherein the combined amount of said iron and said silicon is up to about 0.25 wt %.

60 17. The wrought or cast product of claim 11, further comprising scandium.

18. The wrought or cast product of claim 17, wherein said scandium is present in amount ranging up to about 0.25 wt %.

19. The wrought or cast product of claim 11, further comprising an oxidation-controlling element.

65 20. The wrought or cast product of claim 19, wherein said oxidation-controlling element is beryllium or calcium.

**19**

**21.** The wrought or cast product of claim **11**, wherein said product is an aerospace, sheet, plate, forged or extruded product.

**22.** The aerospace product of claim **21**, wherein said product has a temper selected from the group consisting of T3, 5 T39, T351, T6 and T8.

**23.** A metal matrix composite product made from an aluminum-based alloy having enhanced damage tolerance consisting essentially of:

about 3.0 to about 4.0 wt % copper;  
about 0.4 to about 1.1 wt % magnesium;  
from about 0.2 to about 0.8 wt % silver;

10

**20**

up to about 0.6 wt % Zn, wherein the zinc is partially substituted for the silver and a combined amount of zinc and silver is up to about 0.9 wt %;

up to about 0.25 wt % Zr;

up to about 0.9 wt % Mn;

a combined Fe and Si content of tip to about 0.25 wt % or less Si;

the balance substantially aluminum, incidental impurities and elements, said copper and magnesium present in a ratio of about 3.6-4.5 parts copper to about 1 part magnesium.

\* \* \* \* \*